

3,199,943

PROCESS FOR LOWERING THE SWELLING IN  
WATER OF VISCOSE CELLULOSE BY CYANO-  
ETHYLATION IN THE PRESENCE OF SPECIFIC  
ALKALI METAL SALTSPieter Paulusma, Arnhem, Netherlands, assignor to Ameri-  
can Enka Corporation, Enka, N.C., a corporation of  
Delaware

No Drawing. Filed Oct. 3, 1962, Ser. No. 228,025

Claims priority, application Netherlands, Oct. 9, 1961,

270,070

9 Claims. (Cl. 8—116.2)

This invention relates generally to the production of improved regenerated cellulose products and more particularly to a process for lowering the degree of swelling of regenerated cellulose products in water, especially viscose rayon fibers and fabrics.

It is known that the degree of swelling of regenerated cellulose products in water can be changed by successively treating them with an aqueous solution of an alkali metal hydroxide and acrylonitrile. However, by this process the degree of swelling of, for example, rayon staple fibers, is substantially increased. While such a relatively high degree of swelling may be favorable when the staple fibers are used in guaze bandages or analogous products, it is generally not desirable. Under most circumstances staple fibers or threads of regenerated cellulose should have a relatively low swelling value, particularly if they are processed into woven or knitted fabrics. This is because the dimensions of woven and knitted fabrics of regenerated cellulose yarns are, as is known, less stable than fabrics made of cotton fibers, which have a lower degree of swelling in water than do staple fibers or threads of regenerated cellulose.

It is therefore an object of this invention to provide regenerated cellulose products that have a low degree of swelling in water.

Another object of this invention is to provide a process for treating regenerated cellulose products to lower their degree of swelling in water.

Still another object of this invention, is to provide a process for producing regenerated cellulose products that absorb less moisture from the atmosphere.

These and other objects will become apparent from the following detailed disclosure.

In accordance with applicant's invention, regenerated cellulose products are first treated with an aqueous hydroxide solution that has a normality not higher than 0.70 and contains at least one salt of an alkali metal hydroxide and an inorganic acid derived from one of the first five anions of the lyotropic series according to Hofmeister (see E. A. Hauser, "Colloidal Phenomena," page 132, First Edition, 1939). Thereafter, the products are treated with an azeotropic mixture of acrylonitrile and water. Regenerated cellulose products which may be so treated include threads, staple fibers, woven fabrics, knitted fabrics, films, tapes, foils and products entirely or partly made thereof.

By treating regenerated cellulose products in accordance with applicant's invention, the degree of swelling of such products in water may be reduced from an original value in their untreated state of 75 to, for example, 55. The degree of swelling in this case is determined from the following formula:

$$\frac{B-A}{A} \times 100\%$$

where A is the weight of the air dried cellulose product and B is the weight of the product after it had been soaked in water for two hours and centrifuged for ten minutes.

Surprisingly, if the normality of the hydroxide solution is higher than 0.70, the treated products have a

higher degree of swelling than do the untreated products. Thus, in order to obtain low swelling products, the normality of the hydroxide solution must be below 0.70. Moreover, applicant has discovered that the decrease in degree of swelling of treated products increases as the normality of the caustic solution decreases.

The alkaline metal hydroxides that may be used in the process include lithium hydroxide, sodium hydroxide, potassium hydroxide, rubidium hydroxide, and cesium hydroxide. However, for economy reasons, it is preferred to use sodium hydroxide. The salts added to the caustic solution may be lithium salt, sodium salt, potassium salt, rubidium salt, or cesium salt, although, also for economy reasons, it is preferred to use sodium salts. The salts are derived from an alkali metal hydroxide and any one of the following acids: sulfuric acid, hydrofluoric acid, nitric acid, hydrochloric acid, and hydrobromic acid. The anions of these acids are the first five members of the lyotropic series according to Hofmeister. Preferably, sodium sulphate or sodium chloride is added to the caustic solution since these salts are commercially available at a low price.

It has been found that the reaction may be accelerated by increasing the amount of salt in the caustic solution, the amount of salt added being dependent on the desired decrease in the degree of swelling in the product treated. The temperature at which the treatment with the hydroxide solution is carried out may vary between wide limits. However, higher temperatures are desirable since the wet strength of the product decreases to a lesser extent. Also, the time during which the products are treated with the hydroxide solution preferably should be as short as possible to limit the decrease in the wet strength of the product. If needed, a wetting agent may be added to the hydroxide solution.

After the products have been treated with the hydroxide solution, excess liquid may be removed by centrifuging or pressing. The products are then treated with a mixture of acrylonitrile and a small amount of water. The temperature of the acrylonitrile mixture is maintained as high as possible in order that the treatment may be short, thus allowing the process to be carried out in a continuous manner. For example, the treatment may be carried out at 70° C. using an azeotropic mixture consisting of 88% of acrylonitrile and 12% water. If the treatment is carried out under pressure, even higher temperatures may be used. Alternatively, a mixture of acrylonitrile and a diluent, such as benzene, toluene, acetone, or chloroform may be used. The amount of acrylonitrile reacting with the products may vary within wide limits depending on the decrease in the degree of swelling desired.

Products treated in accordance with this invention not only have a lower degree of swelling in water, but also absorb less moisture in air. As a result of the treatment, the percentage of moisture absorbed from air may be reduced to below 8% which corresponds to a moisture absorption of about 12% for untreated products of regenerated cellulose in air at 20° C. and a relative humidity of 65%.

The invention will be more clearly understood from the following examples. However, these examples are not to be construed as limitative. Percentages are given by weight unless otherwise indicated.

## EXAMPLE I

Viscose rayon staple fibers having a denier of 1½ were separated into several samples and each sample treated with an aqueous sodium hydroxide and salt solution. The normality of the sodium hydroxide solutions varied. Each contained 5% of sodium sulphate. The temperature of the solutions was 90° C. In all cases the treat-

ment lasted one minute. After the treatment each sample was centrifuged and weighed. Thereafter, the samples were treated with acrylonitrile containing 2% water at 20° C. With the exception of run 4, the duration of the treatments was such that equal percentages of acrylonitrile were bound to all samples. The reaction between the regenerated cellulose and acrylonitrile to produce a cyanoethylated product may be expressed by the following equation:



The percentage acrylonitrile bound to the regenerated cellulose is calculated by determining the amount of nitrogen in the dry final product according to the well-known Kjeldahl method. From the amount of nitrogen present in the final product, the number of cyanoethyl groups may be determined and such determination expressed as the weight percent of acrylonitrile bound to the final product. After the treatment with acrylonitrile, the samples were successively washed with dilute acetic acid and warm water and then dried.

The degree of swelling was determined from the formula:

$$\frac{B-A}{A} \times 100\%$$

where A is the weight of the air dried fibers and B is the weight of the fibers immediately following soaking in water for two hours and centrifuging for 10 minutes.

The conditions and results of runs 1 to 10 are set forth in Table I.

respectively. Run 10 shows that potassium hydroxide has the same effect as sodium hydroxide.

#### EXAMPLE II

Samples of staple fibers from the same batch as those of Example I were treated with a sodium hydroxide and salt solution in a manner analogous to that of Example I. In runs 11 to 15, however, the sodium sulphate content was varied. The fibers pre-treated with the sodium hydroxide solution were then treated with an azeotropic mixture of 88% by weight acrylonitrile and 12% by weight water at about 70° C. In runs 16 to 21 salts other than sodium sulfate were added to the sodium hydroxide solution. In run 22 the temperature of the caustic solution was 20° C. The results are set forth in Table II.

Runs 11 to 15 show that by increasing the sodium sulphate content the reaction is considerably accelerated. Runs 16 to 19 show the effects obtained using sodium chloride, potassium sulfate, sodium nitrate, and sodium fluoride as the salts added to the caustic solution. As shown in runs 20 and 21, salts which are not derived from the first five anions of the lyotropic series no longer effect a decrease in the degree of swelling of the fibers. In run 22 the disadvantage of using a low hydroxide solution temperature is shown. Thus, the use of a low temperature in the treatment yields fibers of considerably lower strength than does the use of a high temperature.

#### EXAMPLE III

A fabric having a warp consisting of 120 denier continuous filament viscose rayon threads and a weft consist-

Table I

|         | Hydrox-ide | Normal-ity of hydroxide solution | Salt                            | Percent salt in hydroxide solution | Temp. hydroxide solution, °C. | Hydrox-ide solution treatment time (minutes) | Percent increase in weight after centrifuging | Tempera-ture acrylonitrile/ H <sub>2</sub> O, °C. | Acryloni-trile treat-ment time (minutes) | Percent acryloni-trile bound to fibers | Deg. of swelling in water | Wet strgh., g./d. | Moisture absorption in air at 20° C. R.H. 65% |
|---------|------------|----------------------------------|---------------------------------|------------------------------------|-------------------------------|----------------------------------------------|-----------------------------------------------|---------------------------------------------------|------------------------------------------|----------------------------------------|---------------------------|-------------------|-----------------------------------------------|
| Control |            |                                  |                                 |                                    |                               |                                              |                                               |                                                   |                                          |                                        | 75                        | 102               |                                               |
| 1       | NaOH       | 0.10                             | Na <sub>2</sub> SO <sub>4</sub> | 5                                  | 90                            | 1                                            | 40                                            | 20                                                | 720                                      | 19                                     | 55                        | 71                | 11.7                                          |
| 2       | NaOH       | 0.20                             | Na <sub>2</sub> SO <sub>4</sub> | 5                                  | 90                            | 1                                            | 50                                            | 20                                                | 240                                      | 19                                     | 58                        | 59                | 7.8                                           |
| 3       | NaOH       | 0.50                             | Na <sub>2</sub> SO <sub>4</sub> | 5                                  | 90                            | 1                                            | 65                                            | 20                                                | 150                                      | 19                                     | 60                        | 50                | 7.7                                           |
| 4       | NaOH       | 0.50                             | Na <sub>2</sub> SO <sub>4</sub> | 5                                  | 90                            | 1                                            | 63                                            | 20                                                | 240                                      | 35                                     | 44                        | 38                | 6.1                                           |
| 5       | NaOH       | 0.70                             | Na <sub>2</sub> SO <sub>4</sub> | 5                                  | 90                            | 1                                            | 73                                            | 20                                                | 110                                      | 19                                     | 71                        | 46                | 7.7                                           |
| 6       | NaOH       | 0.80                             | Na <sub>2</sub> SO <sub>4</sub> | 5                                  | 90                            | 1                                            | 80                                            | 20                                                | 90                                       | 19                                     | 95                        | 41                | 7.8                                           |
| 7       | NaOH       | 1.0                              | Na <sub>2</sub> SO <sub>4</sub> | 5                                  | 90                            | 1                                            | 89                                            | 20                                                | 80                                       | 19                                     | 126                       | -----             | 7.9                                           |
| 8       | NaOH       | 1.6                              | Na <sub>2</sub> SO <sub>4</sub> | 5                                  | 90                            | 1                                            | 130                                           | 20                                                | 40                                       | 19                                     | 187                       | -----             | 7.6                                           |
| 9       | NaOH       | 2.5                              | Na <sub>2</sub> SO <sub>4</sub> | 5                                  | 90                            | 1                                            | 241                                           | 20                                                | 15                                       | 19                                     | 211                       | -----             | 7.8                                           |
| 10      | KOH        | 0.5                              | Na <sub>2</sub> SO <sub>4</sub> | 5                                  | 90                            | 1                                            | 42                                            | 30                                                | 300                                      | 19                                     | 60                        | -----             | -----                                         |

Table II

|         | Hydrox-ide | Normal-ity of hydroxide solution | Salt                             | Percent salt in hydroxide solution | Hydrox-ide solution temp., °C. | Hydrox-ide solution treatment time (minutes) | Percent increase in weight after centrifuging | Tempera-ture acrylonitrile/ water, °C. | Acryloni-trile treatment time (minutes) | Percent acryloni-trile bound to fibers | Deg. of swelling in water | Wet strength, g./d. |
|---------|------------|----------------------------------|----------------------------------|------------------------------------|--------------------------------|----------------------------------------------|-----------------------------------------------|----------------------------------------|-----------------------------------------|----------------------------------------|---------------------------|---------------------|
| Control |            |                                  |                                  |                                    |                                |                                              |                                               |                                        |                                         |                                        | 75                        | 102                 |
| 11      | NaOH       | 0.1                              | Na <sub>2</sub> SO <sub>4</sub>  | 1                                  | 90                             | 1                                            | 40                                            | 70                                     | 5                                       | 6.7                                    | 6.7                       | 68                  |
| 12      | NaOH       | 0.1                              | Na <sub>2</sub> SO <sub>4</sub>  | 5                                  | 90                             | 1                                            | 39                                            | 70                                     | 5                                       | 15.9                                   | 60                        | 70                  |
| 13      | NaOH       | 0.1                              | Na <sub>2</sub> SO <sub>4</sub>  | 10                                 | 90                             | 1                                            | 41                                            | 70                                     | 5                                       | 17.2                                   | 58                        | -----               |
| 14      | NaOH       | 0.1                              | Na <sub>2</sub> SO <sub>4</sub>  | 15                                 | 90                             | 1                                            | 43                                            | 70                                     | 5                                       | 18.7                                   | 55                        | -----               |
| 15      | NaOH       | 0.1                              | Na <sub>2</sub> SO <sub>4</sub>  | 20                                 | 90                             | 1                                            | 44                                            | 70                                     | 5                                       | 19.1                                   | 55                        | -----               |
| 16      | NaOH       | 0.1                              | NaCl                             | 5                                  | 90                             | 1                                            | 44                                            | 70                                     | 5                                       | 12.2                                   | 66                        | -----               |
| 17      | NaOH       | 0.1                              | K <sub>2</sub> SO <sub>4</sub>   | 5                                  | 90                             | 1                                            | 45                                            | 70                                     | 5                                       | 13.4                                   | 60                        | -----               |
| 18      | NaOH       | 0.1                              | NaNO <sub>3</sub>                | 5                                  | 90                             | 1                                            | 41                                            | 70                                     | 5                                       | 16.6                                   | 59                        | -----               |
| 19      | NaOH       | 0.1                              | NaF                              | 5                                  | 90                             | 1                                            | 38                                            | 70                                     | 5                                       | 20.6                                   | 51                        | -----               |
| 20      | NaOH       | 0.2                              | KI                               | 46                                 | 90                             | 1                                            | 96                                            | 70                                     | 2½                                      | 23.1                                   | 88                        | -----               |
| 21      | NaOH       | 0.1                              | Na <sub>2</sub> HPO <sub>4</sub> | 25                                 | 90                             | 1                                            | 44                                            | 70                                     | 5                                       | 0.4                                    | 75                        | -----               |
| 22      | NaOH       | 0.1                              | Na <sub>2</sub> SO <sub>4</sub>  | 5                                  | 20                             | 1                                            | 44                                            | 70                                     | 5                                       | 16.5                                   | 60                        | 52                  |

The table shows that using a sodium hydroxide solution having a normality of 0.7 or lower results in a decrease of swelling. The untreated control fibers had a degree of swelling of 75. Fibers treated according to runs 1 to 5 had a degree of swelling of 55, 58, 60, 44 and 71,

respectively. A yarn made of 1½ denier viscose rayon staple fibers, was passed through an aqueous bath maintained at 90° C. containing 1% by weight sodium hydroxide and 5% by weight sodium sulfate. The residence time of the fabric in the bath was one minute. Excess liquid was re-

moved from the fabric by means of pressure rollers. The fabric was then passed through a bath maintained at about 70° C., containing 88% by weight acrylonitrile and 12% by weight water. The residence time of the fabric in this bath was 2 minutes. Excess liquid was removed from the fabric by means of pressure rollers and the fabric was then successively treated with dilute acetic acid and warm water. Thereafter, the fabric was dried. The weight of the treated fabric was 124.7% of its original weight. The fabric was immersed in water and afterwards centrifuged. It then contained about 63% by weight water. A similar sample of untreated fabric, after wetting and centrifuging, contained about 97% by weight water.

## EXAMPLE IV

A self-supporting film made from viscose was passed through an aqueous bath maintained at 90° C. containing 1% by weight sodium hydroxide and 5% by weight sodium sulfate. The residence time of the film in the bath was one minute. The film was passed between two rollers thereby removing excess liquid. Thereafter, the film was passed through a bath maintained at 70° C. containing 88% by weight acrylonitrile and 12% by weight water. Residence time in this bath was 1½ minutes. The film thus treated was passed between two rollers to remove excess liquid and successively washed with dilute acetic acid and warm water. After drying the film was immersed in water and centrifuged. The increase in weight of the film was only 65% in contrast with untreated film, similarly immersed in water and centrifuged which increased 98% in weight.

Various modifications and changes within the scope of the invention will be apparent to those skilled in the art. Therefore, the invention is intended to be limited only as set forth in the following claims.

What is claimed is:

1. A process for lowering the degree of swelling in water of a dry viscose regenerated cellulose product comprising the steps of treating said product with an aqueous solution of an alkali metal hydroxide having a maximum normality of 0.70 for a sufficient period of time to effect cyanoethylation of the product upon subsequent treatment with acrylonitrile, said solution having present therein in addition to said alkali metal hydroxide a small amount of at least one salt of an alkali metal hydroxide and an acid derived from one of the first five anions of the lyotropic series of Hofmeister, treating the alkali impregnated product with acrylonitrile for a sufficient period of time to cyanoethylate the product and to reduce the degree of swelling of the product upon contact with water, and thereafter drying the resulting product.

2. A process for treating a dry viscose regenerated cellulose product to lower its degree of swelling in water comprising the steps of immersing said product in an aqueous solution of an alkali metal hydroxide having a maximum normality of 0.70 for a sufficient period of time to effect cyanoethylation of the product upon subsequent treatment with acrylonitrile, said solution having present therein in addition to said alkali metal hydroxide a small amount of at least one salt of an alkali metal hydroxide and an acid derived from one of the first five anions of the lyotropic series of Hofmeister, immersing the alkali impregnated product in acrylonitrile for a sufficient period of time to bind to the product from about 6.7% to about 35% acrylonitrile, based on the weight of the final cyanoethylated product, and thereafter drying the thus-treated product.

3. A process for treating a dry viscose regenerated cellulose product to lower its degree of swelling in water comprising the steps of immersing said product for about one minute in an aqueous solution of an alkali metal hy-

dioxide having a maximum normality of 0.50 and a temperature of about 90° C., said solution having present therein in addition to said alkali metal hydroxide a small amount of at least one salt of an alkali metal hydroxide and an acid selected from the group consisting of sulfuric acid, hydrofluoric acid, nitric acid, hydrochloric acid, and hydrobromic acid, immersing the alkali impregnated product in an azeotropic mixture of acrylonitrile and water for a sufficient period of time to bind to the product from about 6.7% to about 35% acrylonitrile, based on the weight of the final cyanoethylated product, washing the product, and thereafter drying the thus-treated product.

4. A process for treating a dry viscose regenerated cellulose product to lower its degree of swelling in water comprising the steps of immersing said product for a maximum of two minutes in an aqueous solution of an alkali metal hydroxide having a maximum normality of 0.70, said solution having present therein in addition to said alkali metal hydroxide 5% by weight of said solution of at least one salt of an alkali metal hydroxide and an acid selected from the group consisting of sulfuric acid, hydrofluoric acid, nitric acid, hydrochloric acid, and hydrobromic acid, immersing the alkali impregnated product in an azeotropic mixture of acrylonitrile and water maintained at a temperature ranging from 15° C.-30° C. for a sufficient period of time to bind to the product from about 6.7% to about 35% acrylonitrile, based on the weight of the final cyanoethylated product, washing the product, and thereafter drying the thus-treated product.

5. A process according to claim 4 in which the alkali metal hydroxide is sodium hydroxide and the salt is a sodium salt.

6. The process of claim 5 in which the salt is sodium sulfate.

7. The process of claim 5 in which the salt is sodium chloride.

8. The process of claim 4 in which the regenerated cellulose product is viscose rayon staple fiber.

9. A process for treating a dry viscose regenerated cellulose product to lower its degree of swelling in water comprising the steps of immersing said product in an aqueous solution of an alkali metal hydroxide having a maximum normality of 0.70 for a sufficient period of time to increase the weight of the product by at least 38% after centrifuging, said solution having present therein in addition to said alkali metal hydroxide 5% by weight of at least one salt of an alkali metal hydroxide and an acid selected from the group consisting of sulfuric acid, hydrofluoric acid, nitric acid, hydrochloric acid, and hydrobromic acid, immersing the alkali impregnated product in an azeotropic mixture of acrylonitrile and water maintained at a temperature of 70° C. for a sufficient period of time to bind to the product from about 6.7% to about 35% acrylonitrile, based on the weight of the final cyanoethylated product, washing the product, and thereafter drying the thus-treated product.

## References Cited by the Examiner

## UNITED STATES PATENTS

- |           |       |                         |
|-----------|-------|-------------------------|
| 2,332,049 | 10/43 | Bock et al.             |
| 2,786,735 | 3/57  | Compton et al.          |
| 2,857,239 | 10/58 | Bikales.                |
| 3,018,156 | 1/62  | Bikales.                |
| 3,101,276 | 8/63  | Hendriks ----- 8-116 XR |

## FOREIGN PATENTS

- |         |      |                |
|---------|------|----------------|
| 732,779 | 6/55 | Great Britain. |
| 812,063 | 4/59 | Great Britain. |